

July 2, 1957

M. G. WHITFIELD

2,797,460

CASTING LIGHT METAL AGAINST IRON AND ARTICLE FORMED THEREBY

Filed Sept. 16, 1952

2 Sheets-Sheet 1



**FIG. 1.**



**FIG. 4.**



**FIG. 2.**



**FIG. 5.**



**FIG. 3.**

INVENTOR.  
MARSHALL G. WHITFIELD,  
BY *Allen & Allen*

ATTORNEYS.

July 2, 1957

M. G. WHITFIELD

2,797,460

CASTING LIGHT METAL AGAINST IRON AND ARTICLE FORMED THEREBY

Filed Sept. 16, 1952

2 Sheets-Sheet 2



***FIG. 6.***



***FIG. 7.***

INVENTOR.  
MARSHALL G. WHITFIELD,

BY *Allen & Allen*

ATTORNEYS.

# United States Patent Office

2,797,460

Patented July 2, 1957

1

2,797,460

## CASTING LIGHT METAL AGAINST IRON AND ARTICLE FORMED THEREBY

Marshall G. Whitfield, Garden City, N. Y., assignor to Whitfield & Sheshunoff, Inc., Garden City, N. Y., a corporation of New York

Application September 16, 1952, Serial No. 309,773

7 Claims. (Cl. 22—204)

My invention relates to the problem of producing composite articles of heavy and light metals, of which the formation of aluminum forgings or castings with steel or cast iron inserts will serve as an illustration. For example, it has been proposed to make aluminum pistons with grooved cast iron inserts of annular formation to receive the rings with which the piston will be used in service. Great difficulty has hitherto been encountered in forming a satisfactory and satisfactorily permanent bond between the aluminum and the iron.

Efforts have been made to secure bond by mechanically roughening, knurling or grooving the iron inserts, but without effecting satisfactory results. The procedure of first coating the iron insert by hot-dipping with aluminum has been proposed, and in this connection the employment of various preliminary coatings on the iron of metals more readily wet by the molten aluminum has been suggested. Typical patents in this field are the Whitfield et al. Patent 2,396,730 and Deputy 1,897,689.

The teachings of this application relate to light metals which are to be bonded to ferrous bodies. The light metals are inclusive of magnesium, aluminum, alloys of magnesium and aluminum, and alloys of aluminum, by which I mean alloys consisting preponderantly of aluminum but including other metallic ingredients such as silicon, copper, nickel, iron, vanadium and others or combinations of them. Hereinafter I shall describe my invention in connection with aluminum or aluminum alloys in certain specific embodiments, its application to other light metals being obvious in the light of the foregoing. By ferrous bodies I mean to include irons, mild steels, and cast irons, with or without alloying ingredients frequently found in such materials.

A principal object of my invention is the provision of a method which is simple, straightforward and economical for producing a proper bond between a ferrous body and a light metal cast in place. While ordinarily the ferrous body will be located in a mold and a light metal body formed about it by casting, my procedure is inclusive of one where both a ferrous body and a light metal forging or the like are located in a mold and are bonded together by casting molten light metal between the two.

It is an object of my invention to provide a method of forming composite articles in which the problems set forth in what has been said above are solved in a simple and economical fashion.

It is an object of my invention to provide a method of obtaining a new and improved bond between a light metal applied in molten condition and a ferrous body, the bond being of a type not hitherto observed.

It is also an object of my invention to provide a way of forming an excellent bond between a light metal and a ferrous body when the light metal contains substantial quantities of alloying ingredients ordinarily interfering with bond formation.

It is an object of the invention to form a proper bond

2

between a light metal and a ferrous base without the necessity of a hot-dipping procedure.

These and other objects of the invention which will be set forth hereinafter or will be clear to the skilled worker in the art upon reading these specifications, I accomplish by that procedure and in that article of which I shall now describe exemplary embodiments. Reference is made to the accompanying drawings in which Figures 1 to 7 inclusive (hereinafter more fully described) are 10 photomicrographs of structures in which aluminum is bonded to iron.

Briefly, in the practice of my invention, the ferrous body is thinly coated with a metal easily wetted by molten aluminum or other light metal, the body is then 15 located in a mold wherein it is at an elevated temperature but below the melting temperature of the metal being cast against it. The molten light metal is then caused to flow into the mold and over the surfaces of the ferrous body to which it is to be bonded in such fashion that there is a substantial flow of the molten metal past these surfaces with a flushing action as will hereinafter be explained. These factors will now individually be discussed.

It has been known that in hot-dipping processes aluminum or other light metal will not adequately wet the surface of iron if that surface is covered with oxide. It is necessary in such processes to maintain contact between the molten metal and the iron for a sufficient time to permit the solution or reduction of the oxide. 30 Thereupon wetting occurs and an interface alloy is formed.

It has been suggested that this condition could be ameliorated by first coating the iron with a metal having a lower melting point than the light metal and more readily wet by it than iron. Such metals are in general tin, zinc and cadmium. When one of these metals is plated or otherwise deposited on iron wire, strip or articles prior to hot-dipping a more rapid wetting in a shorter immersion time is effected. The result of immersion, however, is the formation of a coating of the light metal on the ferrous base accompanied by a sharply defined interface alloy layer. In the case of a tin coating on iron which is then hot-dipped in aluminum, the interface alloy layer is probably a tin-iron-aluminum alloy. The alloy layer is somewhat rough on the light metal side of the composite, but usually appears relatively smooth and sharply demarcated on the iron side of the composite.

In the procedures of the patents noted above a ferrous body is first hot-dipped in the molten light metal, after which it is located in a mold and additional light metal cast against it. The casting of additional light metal in molten condition against a previously formed hot-dip coating does not diminish the interface alloy layer, but on the contrary has a tendency to increase its thickness, if anything. While in general in casting procedures better results are secured by casting the light metal against a previously formed hot-dip coating, it has been found that a source of weakness lies in the interface alloy layer. For example, aluminum pistons having cast iron inserts exhibit a fracturing of the bond, either immediately after formation, or after a very short service life. In exaggerated instances, the ferrous body may be entirely loosened from the surrounding light metal casting. In most instances the bond fractures in part only initially, the fracture tending to spread during the service life of the article.

In the practice of my process I employ on the ferrous body a coating of metal such as tin, zinc or cadmium which will promote wetting, but the step of hot-dipping is omitted by control of the other factors mentioned above, when the molten light metal is cast against the ferrous

body ready wetting occurs, but the characteristic hot-dip alloy coating does not appear to be formed. In some instances there is a visual absence of alloy coating when the composite structure is sectioned, etched and viewed under the microscope. In other instances the interface alloy layer appears not only to be diminished in depth but also to have a different form or configuration. The nature of the bond is greatly improved.

The degree of preheat of the ferrous body in the mold will vary with its thickness and the proportion of casting metal to the size of the insert or body. But the body will be heated to a temperature below the melting point of the molten coating metal. One result of this appears to be the formation, in place of or adjacent to the interface alloy layer, of a zone in which alloying constituents of the molten light metal are precipitated in very finely divided condition. Without wishing to be bound by theory, I believe that this effect results from a chilling of the molten metal adjacent the insert or body, and that the formation of a zone of fine precipitation substantially improves the nature of the bond. By this I mean to indicate that, whereas with a highly alloyed light metal (say an aluminum containing large quantities of silicon and/or other metals) more difficulty is ordinarily encountered in forming an adequate bond with iron, a substantially better bond appears to result when there is formed the fine precipitation zone aforesaid.

Another important characteristic of my process is the carrying on of the casting operation in such fashion that the molten metal being cast flows over and around and flushes the surfaces of the metal body or insert for an appreciable interval of time. Again without wishing to be bound by theory, I believe that this flushing action has the effect of breaking up oxide layers which always exist on the surfaces of molten aluminum and magnesium and their alloys even when a non-oxidizing atmosphere is maintained over the plated surfaces of the ferrous bodies. I believe that by the flushing action the surface of the ferrous body are cleansed of occluded gases while any oxides on the surface of the molten light metal are parted, allowing a clean metal-to-metal contact and inter-solution.

Whether the flushing action has any effect on the formation of the interface alloy, or to what extent this is affected by the formation of the fine precipitation zone, or whether the interface alloy is minimized or obviated merely by casting the molten light metal against the relatively cooler surfaces of the ferrous body, is not known. However, after practice of my invention, examination of the interface between the cast metal and the ferrous body indicates that the formation of iron-aluminum alloy is retarded, sometimes suppressed completely, and in other cases reduced to a degree hitherto impossible by known methods taken into account the metals involved.

The flowing or flushing action which has been mentioned above can be attained in various ways, depending in part on the nature of the composite articles being produced. In some instances it is possible so to design the gates and risers of a mold that all of the metal which enters the mold must first pass over the surfaces of the ferrous body or insert. In some instances it is possible to secure the effect of flushing by deliberate agitation of the molten metal by the time it has solidified, so as to cause it to move across the surfaces of the ferrous body. In most instances an adequate effect of flushing can most readily be secured by continuing the pouring after the mold has filled, so that excess metal exits from the risers.

As the casting metal goes past the plated insert of ferrous body, the plated metal, having a lower melting point than the molten casting metal, is caused to flow and initiate a bonding action with the surface metal of the ferrous body. The molten casting metal that finally comes to rest against the ferrous body is, under the preferred conditions of my process, the hottest metal in the casting. This helps in the absorption of the plated metal into the

casting metal and in this way presumably removes a potential source of weakness at the bonding zone.

The above teachings will now be contrasted with prior art procedures, and illustrated by reference to certain examples. Figures 6 and 7 are typical photomicrographs at a magnification of 250 $\times$  of different composite structures. In each of the figures the cast iron is the lowermost layer, and the aluminum the uppermost layer. Between the two there will be seen a sharply demarcated alloy layer, very thick in the case of Figure 7. In each case the cast iron body was electro-tinned, then dip-coated in a molten, high silicon-aluminum bath, followed by casting a high silicon-aluminum alloy against the hot coated surface in a mold. The aluminum alloy was a material produced in accordance with the teachings of the Schwarz Patent 2,131,076, and contained from 21 to 23 percent of silicon together with small amounts of nickel, copper, vanadium and magnesium, the balance being aluminum. The alloy is known as vanasil, and is an advantageous alloy for the formation of pistons for internal combustion engines by reason of its heat expansion characteristics. It may be noted that alloying constituents of the molten coating metal precipitated in large masses adjacent to and sometimes actually inside the interface alloy layer.

The bonds of the articles illustrated in Figures 6 and 7, were found to be functionally deficient.

#### Example 1.

A cylindrical tube with a variable diameter ranging from approximately 1.8 inch to approximately 3 inches, made of low carbon steel and having a thickness of .015 inch was bright annealed in a hydrogen furnace, electro-plated with tin in a conventional alkaline tin plating bath to a thickness of .0002 over the outer surface. Baked sand cores were fitted into the ends of the tube to fill it and support it in an outer mold which was also made of baked sand. The tube was placed in the sand mold, which was so gated that the metal to be cast would flow past and up around the tin plated tube and out the top of the mold. An aluminum alloy (Alcoa 355) at a temperature of 1380° F. was poured into the gate so as to flow past the surface of the tube for approximately 10 to 20 seconds. When the casting had solidified an excellent bond was seen to have developed.

A section of the composite article, etched with nital, is shown in Figure 4 of the drawings. Again the lower layer represents the steel, the upper layer the aluminum alloy and the intermediate layer an alloy bond. The thickness of the alloy bond is substantially diminished as can be seen by comparing Figure 4 with Figure 7, and there is no irregular penetration of the base which commonly occurs with low carbon steel. In this particular article there is no visual indication of a fine precipitation zone. This is believed to be due to the fact that the aluminum alloy used contained only 5 percent silicon, 1.3 percent copper and 0.5 percent magnesium, the balance being aluminum except for normal impurities. It will be seen that there is likewise no indication of coarse precipitation.

#### Example 2

A grey iron ring 5 $\frac{1}{4}$  inch in outside diameter and 4 $\frac{1}{4}$  inch in inside diameter, having a thickness of  $\frac{3}{16}$  inch was plated with tin in an alkaline (sodium stannate) tin bath to a thickness of .00015 inch. It was placed in an iron mold which had been heated to a temperature of about 600 to 700° F.; and when the ring itself had risen in temperature of approximately 400° F., molten high silicon-aluminum alloy at a temperature of about 1525° F. was poured over the ring surfaces on which bonding was desired in such a way that the molten metal flowed over the surfaces of the ring for 5 to 10 seconds. This piston ring insert casting was then placed in an electric heat treating oven for one hour at a temperature of 960° F., cooled in an air blast, placed in an electric oven for three hours at 310° F., and slowly cooled to room temperature.

Figure 1 shows the bond developed, and serves as an example of almost perfect bond control. The sectioned sample was etched in nital and is viewed under a magnification of 250 X. The lower layer is the cast iron insert, the upper layer the aluminum alloy and a fine precipitation zone is clearly apparent between the two. The aluminum alloy was the vanasil mentioned above. The sample shows no visual evidence of the typical iron-aluminum interface alloy layer. Instead there lies above the iron a layer of aluminum containing its alloying constituents precipitated in a very fine state of subdivision.

#### Example 3

Figure 2 is a photomicrograph at 250 X magnification of a section of a similar structure similarly treated except that the conditions were not so carefully controlled. Here again vanasil was cast against an electro-tined cast iron insert ring. In the case of the particular section, a thin layer of recognizable interface alloy is shown overlying the iron lower layer; but there is clearly apparent above it a fine precipitation zone in which the alloying constituents appear in finely divided form. The bond produced in the article sectioned in Figure 2 was tested and found to be highly satisfactory.

Figure 2 is an illustration of the fact that relatively slight variations in temperature or in the volume and duration of the flow of molten metal past a surface to which it is to be bonded, will produce visual variations in the bond itself. Moreover in different parts of a given mold, or in different areas of the surface of a given insert there may occur variations in temperature and in volume flow of the molten metal which will produce visual differences in the bond. The best possible results appear to be attained when the ferrous insert or body is heated so that the coating of tin, zinc or cadmium on its surface is rendered fluid in the presence of an inert or reducing gas such as argon, helium or hydrogen, and when the greatest possible volume of flow of the molten light metal or alloy over the surfaces of the insert or body is attained. Even with the variations which have been noted, however, the teachings herein set forth will produce a bond which is mechanically adequate, and far superior to any bond which has hitherto been produced by other procedures.

#### Example 4

A composite article was produced by the method outlined in connection with Examples 2 and 3 excepting that the cast iron body was electroplated with cadmium instead of tin and the aluminum alloy which was cast against it contained only 12 percent of silicon instead of the 21 to 23 percent characteristic of the vanasil mentioned above. Figure 3 is a nital etched section at a magnification of 250 X. The cast iron is the lower layer and the aluminum alloy the top layer. Between the two there will be seen some slight evidence of an alloy interface. In spite of the lower content of silicon a fine precipitation zone is clearly apparent. The bond was good.

#### Example 5

Two circular steel sheets approximately .10 inch thick were electroplated with tin to a thickness of about .0001 inch and were placed in a mold adjacent to an alloy aluminum forging which had been preheated to a temperature approximately 100° F. below the melting point of the aluminum alloy, under an atmosphere of argon or helium and molten aluminum alloy of the same analysis as the forging and at a temperature of approximately 1400° F., was poured into the mold so as to flow over the tin-plated surfaces of the iron bodies, filling the space between the sheets and the preheated forging, bonding to both simultaneously. The aluminum alloy was one known as 7-5 and contained 5 percent silicon, 7 percent copper and .5 percent nickel. The bond was good.

#### Example 6

An iron insert was electroplated with zinc, and was

then heated in a protective atmosphere (to minimize oxidation of the plated layer) to a temperature a little above the melting point of zinc. An aluminum alloy containing 5 percent silicon, 7 percent copper and 0.5 percent nickel at a temperature of 1375° F. was poured over the insert. In this instance, because of the preheating and lack of oxide on the surface of the electroplated layer, no overfilling of the mold was employed.

A nital etched section through the insert and the adjacent aluminum alloy (250 X) is shown in Figure 5. Here there is no visual evidence of a fine precipitation zone and, while irregular, there is a sharply defined alloy interface layer. A better bond was produced than was characteristic of the hot-dipped procedures of the prior art, although the bond was not as good as that, for example, of Figure 1.

The conclusions which I have reached in the development herein outlined are that superior bonds can be attained between a ferrous body and a cast light metal structure if instead of hot-dipping the ferrous body the light metal is so cast against it as to flush the surface of the ferrous body for an appreciable interval of time. The use of a plated coating of tin, zinc, cadmium or the like greatly promotes wetting but is not sufficient to assure a good bond with cast light metal in the absence of the flushing action which has been described. Preheating the ferrous body in a non-oxidizing or reducing atmosphere appears to help in preventing lack of wetting by reason of oxides interposed between the molten light metal and the ferrous body, and to this extent is a partial substitute for the flushing action. But inasmuch as the flushing action will produce a superior bond to that produced when the molten light metal is simply cast against the plated surface of the ferrous body even though that surface was treated in and protected by a reducing atmosphere, the flushing action is more properly regarded as a primary inexpensive and extremely effective way of eliminating oxide films which prevent wetting. The particular preferred conditions outlined result in a new type of bond characterized by a diminution and in some instances elimination of the alloy interface. A chilling of the molten metal resulting from a lower temperature of the ferrous body is of advantage in promoting bond by causing a finely divided precipitation of alloying constituents in the light metal, and this is of especial value when the quantity of alloying constituents such as silicon, copper, nickel, vanadium and the like is large. The temperature of the iron body, considering its mass should not be so low that a plated coating of tin, cadmium or zinc cannot be raised above its melting point by heat from the molten light metal. With this lower limitation, however, the advantage appears to lie with lower temperatures of preheat of the ferrous body rather than temperatures approaching that of the molten coating metal. The visual appearance of a fine precipitation zone is apparent in my etched samples only when the quantity of alloying constituents present is fairly high; but I believe that the value of the fine precipitation of alloying constituents extends to fairly low quantities, and that the chilling effect is worth while at least down to contents of 5 percent silicon or less.

Modifications may be made in my invention without departing from the spirit of it. Having thus described my invention in certain exemplary embodiments, what I claim as new and desire to secure by Letters Patent is:

65 1. A process of casting a light metal against a ferrous body which comprises electroplating the said ferrous body with a wetting metal chosen from a class consisting of tin, zinc and cadmium, locating the ferrous body in a mold, the said body being heated to a temperature approaching but below the melting point of the light metal which is to be cast thereagainst, said temperature being chosen in the light of the effective mass of the said ferrous body, the temperature of the light metal and the length of time of the casting operation, so that during the casting operation the said wetting metal will be

liquefied while at the same time the said ferrous body will produce a chilling action on the light metal cast thereagainst, and casting against the said treated ferrous body a light metal chosen from a class consisting of aluminum and alloys of aluminum and other metals in which alloys, aluminum is preponderant, and causing the molten light metal to flow against and past, and flush the exposed surfaces of the ferrous body for a sufficient length of time to remove oxide films between the light metal and the surfaces of the ferrous body and carry 10 the said oxide films away from the ferrous body.

2. The process claimed in claim 1 in which the flushing action is accomplished by providing entrance and exit means in connection with the mold, so locating these that metal issuing from the exit means must have flowed 15 over the surfaces of the ferrous body, and continuing the pouring for a substantial interval after the mold has been filled.

3. The process claimed in claim 2 in which the said wetting metal is tin.

4. The process claimed in claim 3 wherein said light metal is an aluminum alloy rich in silicon, said chilling action serving to cause finely divided precipitation of the said silicon adjacent the interface between the ferrous body and the light metal cast thereagainst.

5. The process claimed in claim 4 wherein the article so formed is a light metal piston and the said ferrous body is an insert therein.

6. A composite article produced in accordance with claim 1.

7. A composite article produced in accordance with claim 4.

#### References Cited in the file of this patent

#### UNITED STATES PATENTS

|           |                   |               |
|-----------|-------------------|---------------|
| 286,459   | McCarthy          | Oct. 9, 1883  |
| 534,979   | Stark             | Feb. 26, 1895 |
| 1,043,577 | Eldred            | Nov. 5, 1912  |
| 1,528,947 | Preston           | Mar. 10, 1925 |
| 1,669,071 | Thomas            | May 8, 1928   |
| 1,732,515 | Hunter            | Oct. 22, 1929 |
| 1,738,056 | Hunter            | Dec. 3, 1929  |
| 1,938,707 | Mann              | Dec. 12, 1933 |
| 2,265,243 | McCullough et al. | Dec. 9, 1941  |
| 2,435,991 | Whitfield         | Feb. 17, 1948 |
| 2,544,670 | Grange et al.     | Mar. 13, 1951 |
| 2,544,671 | Grange et al.     | Mar. 13, 1951 |
| 2,634,469 | Pershing et al.   | Apr. 14, 1953 |
| 2,672,666 | Enfer et al.      | Mar. 23, 1954 |

#### FOREIGN PATENTS

|         |               |               |
|---------|---------------|---------------|
| 351,977 | Great Britain | June 25, 1931 |
| 428,586 | Great Britain | May 15, 1935  |
| 634,599 | Great Britain | Mar. 22, 1950 |

#### OTHER REFERENCES

Metal Handbook, 1948 edition, p. 11, published by The American Society for Metals, 7301 Euclid Ave., Cleveland, Ohio.